

June 15, 1926.

1,589,013

H. S. LEE

METHOD OF ANNEALING METAL

Filed August 27, 1924



Inventor

Harry S. Lee

By *Stuart C Barnes*

Attorney

## UNITED STATES PATENT OFFICE.

HARRY S. LEE, OF PLYMOUTH, MICHIGAN.

## METHOD OF ANNEALING METAL.

Application filed August 27, 1924. Serial No. 734,404.

This invention relates to a method of self-annealing metals and is especially adapted for annealing grey iron castings made in permanent or cast iron moulds. To prevent castings from oxidizing and to prevent the formation of a scale thereon, it is necessary to prevent the casting from coming in contact with the atmosphere while the same is cooling. This invention prevents the casting and the oxygen in the atmosphere from coming into contact.

Castings which are made in permanent moulds are very often chilled. This chilling is caused by the metal of the casting contacting with the cast iron of the mould and cooling more quickly at the surface than in the interior. This chilling changes the chemical structure of the outer surface of the casting, and the chilled portion of the casting becomes very hard, and makes the machining of the casting difficult.

Another disadvantage of a chilled casting is that it does not allow the metal to be relieved of internal strains so that when the metal is machined to size it retains its dimensions and shape.

A feature of my process is the self-annealing of the casting by its own heat. The casting is precipitated into the annealing compound while it is at the annealing temperature or just solidified and the heat of the casting itself is confined therein and performs the annealing operation.

To illustrate this method, I have chosen to diagrammatically illustrate a mechanism for performing the method, though the different steps in the method can obviously be performed by hand.

In the drawings:

Fig. 1 is a diagrammatic view of a system.

Fig. 2 is an enlarged section through my annealing tank, showing how my annealing material entirely covers the casting precipitated in the tank.

The description of the apparatus is simple. *a* designates any furnace which may be used for melting the metal, from which the molten metal is poured into the moulds *b*, which are traveling on a continuous belt or conveyor *c*, driven from any suitable source of power and here shown as a motor *M*. This conveyor will convey the moulded castings to a point remote from the furnace, and means may be provided for auto-

matically ejecting the casting from the mould and precipitating the same into an annealing tank *d*. Obviously, these moulds could be opened manually and the casting pushed out by a tool to precipitate the same in the tank.

My annealing tank is filled with a quantity of powdered kieselguhr, diamataceous earth or infusorial earth. The characteristic of this kieselguhr is that it is a very efficient heat insulator, and prevents the escape of the heat from the heated casting that is dropped therein to the outside atmosphere. This finely powdered kieselguhr is like dust and acts in a way similar to quicksand. As the casting is dropped into the bath of kieselguhr it quickly sinks into the ground kieselguhr, the kieselguhr closing about the casting and effectively excluding the oxygen in the atmosphere from the casting. The kieselguhr beneath the casting is packed sufficiently by the weight of the casting so as to provide a pad of kieselguhr of several inches in thickness.

I may or may not use a little powdered fire clay. When using this finely powdered fire clay together with the kieselguhr, I preferably use a mixture of about 10% fire clay to 90% kieselguhr.

This kieselguhr possesses the characteristics of preventing the heat of the casting from escaping and as a result of my experiments I find that a heated casting that is immersed in this material and kept therein for 24 hours is still too hot to be handled by hand. The internal heat of the casting performs the annealing. As a result, this annealing bath of kieselguhr forms a very good annealing material as it enables one to cool the casting very, very slowly and in addition effectively prevents oxygen from coming in contact with the casting while so cooling in the process of self-annealing.

What I claim is:

The method of treating castings, which comprises dropping them while at a relatively high temperature into a powdered heat-insulating medium in which kieselguhr predominates, said heat-insulating medium being of a depth calculated to substantially completely cover the casting.

In testimony whereof I have affixed my signature.

HARRY S. LEE.